



US012006586B2

(12) **United States Patent**  
**Räisä et al.**

(10) **Patent No.:** **US 12,006,586 B2**  
(b4) **Date of Patent:** **Jun. 11, 2024**

(54) **OBJECT COMPRISING A CHROMIUM-BASED COATING WITH A HIGH VICKERS HARDNESS, PRODUCTION METHOD, AND AQUEOUS ELECTROPLATING BATH THEREFOR**

2017/0009361 A1 1/2017 Dal Zilio et al.  
2017/0159198 A1 6/2017 Miettinen et al.  
2019/0040540 A1 2/2019 Raisa  
2019/0309430 A1 10/2019 Sklar  
2021/0017659 A1\* 1/2021 Ijeri ..... C25D 3/56

(71) **Applicant:** **Savroc Ltd**, Kuopio (FI)

CN 101392394 3/2009

(72) **Inventors:** **Jussi Räisä**, Kuopio (FI); **Arto Yli-Pentti**, Klaukkala (FI)

CN 101410556 4/2009

(73) **Assignee:** **Savroc Ltd**, Kuopio (FI)

CN 105297084 11/2018

(\*) **Notice:** Subject to any disclaimer, the term of this patent is extended or adjusted under 35 U.S.C. 154(b) by 0 days.

EP 0073221 3/1983

EP 2980280 2/2016

FR 2331628 6/1977

GB 1482747 8/1977

GB 1592761 7/1981

WO 2016044708 3/2016

WO 2021214389 10/2021

**FOREIGN PATENT DOCUMENTS**

(21) **Appl. No.:** **17/996,632**

**OTHER PUBLICATIONS**

(22) **PCT Filed:** **Apr. 21, 2021**

ASTM G195-18 (Year: 2018).\*

(86) **PCT No.:** **PCT/FI2021/050297**

“FI Search Report for 20205408”, dated Oct. 2, 2020, 1 pg.

§ 371 (c)(1),  
(2) Date: **Oct. 20, 2022**

“PCTFI20211050297 International Search Report and Written Opinion dated Jun. 30, 2022”, Jun. 30, 2021, 15 pgs.

(87) **PCT Pub. No.:** **WO2021/214389**

Benaben, P., “Thick, Hard Electrodeposits From a Trivalent Chromium Bath”, Electroplaters Society, Inc., East Orange, US, vol. 76, No. 11, Nov. 1, 1989 (Nov. 1, 1989), pp. 60-63, XP000083921, ISSN: 0360-3164, table 2 p. 61, left-hand column, paragraph 3rd Nov. 1, 1989, 4 pgs.

PCT Pub. Date: **Oct. 28, 2021**

Huang, Ching A. et al., “Anneal-hardening behaviour of CrC, CrNiC and CrNiFeC alloy deposits”, Journal of the Taiwan Institute of Chemical Engineers, vol. 96, Mar. 1, 2019 (Mar. 1, 2019), pp. 543-548, XP085614485, ISSN: 1876-1070, DOI: 10.1016/j.jtice.2018.11.005 Mar. 1, 2019, 6 pgs.

(65) **Prior Publication Data**

Huang, Ching A. et al., “Microstructure and electrochemical corrosion behavior of Cr—Ni—Fe alloy deposits electroplated in the presence of trivalent Cr ions”, Thin Solid Films, vol. 544, Oct. 1, 2013 (Oct. 1, 2013), pp. 69-73, P055316775, Amsterdam, NL ISSN: 0040-6090, DOI: 10.1016/j.tsf.2013.04.124, Section 4: Conclusion Oct. 1, 2013, 5 pgs.

US 2023/0129051 A1 Apr. 27, 2023

“CN Application No. 202180030113.4 Office Action”, dated Apr. 17, 2023, 17 pages.

(30) **Foreign Application Priority Data**

(Continued)

Apr. 23, 2020 (FI) ..... 20205408

**Primary Examiner** — Wojciech Haske

(51) **Int. Cl.**

(74) **Attorney, Agent, or Firm** — DeLizio, Peacock, Lewin & Guerra

**C25D 3/06** (2006.01)  
**C25D 3/10** (2006.01)  
**C25D 5/00** (2006.01)  
**C25D 5/14** (2006.01)  
**C25D 3/14** (2006.01)

(52) **U.S. Cl.**

**ABSTRACT**

CPC ..... **C25D 3/06** (2013.01); **C25D 3/10** (2013.01); **C25D 5/14** (2013.01); **C25D 5/617** (2020.08)

An object comprising a chromium-based coating on a substrate is disclosed, wherein the chromium is electroplated from an aqueous electroplating bath comprising trivalent chromium cations, wherein the chromium-based coating comprises 87-98 weight-% of chromium, 0.3-5 weight-% of carbon, and 0.1-11 weight-% of nickel and/or iron, and wherein the chromium-based coating has a Vickers microhardness value of 1000-2000 HV, and wherein the chromium-based coating does not contain chromium carbide. Further is disclosed a method for its production, and an aqueous electroplating bath.

(58) **Field of Classification Search**

None

See application file for complete search history.

(56) **References Cited**

**U.S. PATENT DOCUMENTS**

4,093,521 A 6/1978 Renton et al.  
4,184,929 A 1/1980 Tomaszewski et al.  
4,690,735 A 9/1987 Laitinen et al.  
5,415,763 A 5/1995 Johnson et al.  
5,759,243 A 6/1998 Johnson  
6,329,071 B1 12/2001 Kobayashi et al.  
7,052,592 B2 5/2006 Edigaryan  
11,795,559 B2 10/2023 Räisä et al.  
2009/0114544 A1\* 5/2009 Rousseau ..... C25D 3/10  
205/243

2015/0361571 A1 12/2015 Miettinen et al.  
2016/0318282 A1 11/2016 Muchtar et al.

**5 Claims, No Drawings**

(56)

**References Cited**

OTHER PUBLICATIONS

- “CN Application No. 202180030423.6 Office Action”, dated May 23, 2023, 12 pages.
- “U.S. Appl. No. 17/919,688 Office Action”, dated Mar. 13, 2023, 7 pages.
- “U.S. Appl. No. 17/996,642 Office Action”, dated Mar. 29, 2023, 6 pages.
- Oduoza, et al., “Chromium Electroplating of Aluminium Alloys Using Electroless Nickel as Underlayer”, Journal of Materials Science and Chemical Engineering, Jan. 1, 2014—ISSN 2327-6045, vol. 2, Nr:7, pp. 59-74, Jul. 1, 2014, 17.
- “U.S. Appl. No. 17/996,521 Office Action”, dated Nov. 15, 2023, 10 pages.
- “U.S. Appl. No. 17/996,521 Office Action”, Mar. 22, 2024, 7 pages.

\* cited by examiner

## 1

**OBJECT COMPRISING A  
CHROMIUM-BASED COATING WITH A  
HIGH VICKERS HARDNESS, PRODUCTION  
METHOD, AND AQUEOUS  
ELECTROPLATING BATH THEREFOR**

**TECHNICAL FIELD**

The present disclosure relates to an object comprising a chromium-based coating on a substrate. The present disclosure further relates to a method for producing an object comprising a chromium-based coating on a substrate. The present disclosure further relates to an aqueous electroplating bath.

**BACKGROUND**

Objects which are utilized in demanding environmental conditions often require e.g., mechanical or chemical protection, so as to prevent the environmental conditions from affecting the object. Protection to the object can be realized by applying a coating thereon, i.e., on the substrate. Disclosed are protective coatings for various purposes, hard-coatings that protect the substrate from mechanical effects and diffusion barriers for protection against chemical effects. However, further manners to produce hard-coatings in an environmentally friendly manner are needed.

**SUMMARY**

An object comprising a chromium-based coating on a substrate is disclosed. The chromium may be electroplated from an aqueous electroplating bath comprising trivalent chromium cations. The chromium-based coating may comprise 87-98 weight-% of chromium, 0.3-5 weight-% of carbon, and 0.1-11 weight-% of nickel and/or iron. The chromium-based coating may have a Vickers microhardness value of 900-2000 HV. The chromium-based coating does not contain chromium carbide.

An object comprising a chromium-based coating on a substrate is disclosed. The chromium may be electroplated from an aqueous electroplating bath comprising trivalent chromium cations. The chromium-based coating may comprise 87-98 weight-% of chromium, 0.3-5 weight-% of carbon, and 0.1-11 weight-% of nickel and/or iron. The chromium-based coating may have a Vickers microhardness value of 1000-2000 HV. The chromium-based coating does not contain chromium carbide.

Further is disclosed a method for producing an object comprising a chromium-based coating on a substrate. The method may comprise:

depositing a chromium-containing layer on the substrate by subjecting the substrate to at least one electroplating cycle from an aqueous electroplating bath, wherein the electroplating cycle is carried out at a current density of 50-300 A/dm<sup>2</sup> and at a deposition rate of 1.5-10 µm/minute, and wherein the aqueous electroplating bath comprises:

trivalent chromium cations in an amount of 0.12-0.3 mol/l,

iron cations and/or nickel cations in an amount of 0.18-6.16 mmol/l, and

carboxylate ions in an amount of 1.22-7.4 mol/l, and

wherein the molar ratio of trivalent chromium cations to the carboxylate ions is 0.015-0.099, and wherein the pH of the aqueous trivalent chromium bath is 2-6,

## 2

to produce a hard chromium-based coating having a Vickers microhardness value of 900-2000 HV without subjecting the deposited chromium-containing layer to a heat treatment.

5 Further is disclosed an aqueous electroplating bath. The aqueous electroplating bath may comprise:

trivalent chromium cations in an amount of 0.12-0.3 mol/l,

iron cations and/or nickel cations in an amount of 0.18-6.16 mmol/l, and

carboxylate ions in an amount of 1.22-7.4 mol/l, and

wherein the molar ratio of trivalent chromium cations to the carboxylate ions is 0.015-0.099, and wherein the pH of the aqueous trivalent chromium bath is 2-6.

15 Further is disclosed an aqueous electroplating bath. The aqueous trivalent chromium bath may comprise:

trivalent chromium cations in an amount of 0.12-0.3 mol/l,

iron cations and/or nickel cations in an amount of 0.18-6.16 mmol/l, and

carboxylate ions in an amount of 1.2-7.4 mol/l, and

wherein the molar ratio of trivalent chromium cations to the carboxylate ions is 0.015-0.099, wherein the pH of the aqueous trivalent chromium bath is 2-6; and wherein the

25 conductivity of the aqueous electroplating bath is 160-400 mS/cm.

**DETAILED DESCRIPTION**

30 The present disclosure relates to an object comprising a chromium-based coating on a substrate. The chromium may be electroplated from an aqueous electroplating bath comprising trivalent chromium cations. The chromium-based coating may comprise 87-98 weight-% of chromium, 0.3-5 weight-% of carbon, and 0.1-11 weight-% of nickel and/or iron. The chromium-based coating may have a Vickers microhardness value of 900-2000 HV. The chromium-based coating may not contain chromium carbide.

The present disclosure relates to an object comprising a 40 chromium-based coating on a substrate. The chromium may be electroplated from an aqueous electroplating bath comprising trivalent chromium cations. The chromium-based coating may comprise 87-98 weight-% of chromium, 0.3-5 weight-% of carbon, and 0.1-11 weight-% of nickel and/or iron. The chromium-based coating may have a Vickers microhardness value of 1000-2000 HV. The chromium-based coating does not contain chromium carbide.

45 As is clear to the skilled person, the total amount of the different elements in the chromium-based coating may not exceed 100 weight-%. The amount in weight-% of the different elements in the chromium-based coating may vary between the given ranges.

The present disclosure further relates to a method for producing an object comprising a chromium-based coating on a substrate. The method may comprise:

depositing a chromium-containing layer on the substrate

by subjecting the substrate to at least one electroplating

cycle from an aqueous electroplating bath, wherein

each of the at least one electroplating cycles is carried

out at a current density of 50-300 A/dm<sup>2</sup> and at a

deposition rate of 1.5-10 µm/minute, and wherein the

aqueous electroplating bath comprises

trivalent chromium cations in an amount of 0.12-0.3

mol/l,

iron cations and/or nickel cations in an amount of 0.18-

6.16 mmol/l, and

carboxylate ions in an amount of 1.22-7.4 mol/l, and

wherein the molar ratio of trivalent chromium cations to the carboxylate ions is 0.015-0.099, and wherein the pH of the aqueous trivalent chromium bath is 2-6,

to produce a hard chromium-based coating having a Vickers microhardness value of 900-2000 HV without subjecting the deposited chromium-containing layer to a heat treatment.

In one embodiment, the method for producing an object comprising a chromium-based coating on a substrate comprises producing the object comprising a chromium-based coating on a substrate as defined in the current specification.

The present disclosure relates to an aqueous electroplating bath. The aqueous electroplating bath may comprise:

trivalent chromium cations in an amount of 0.12-0.3 mol/l,

iron cations and/or nickel cations in an amount of 0.18-6.16 mmol/l, and

carboxylate ions in an amount of 1.22-7.4 mol/l, and

wherein the molar ratio of trivalent chromium cations to the carboxylate ions is 0.015-0.099, and wherein the pH of the aqueous trivalent chromium bath is 2-6.

The present disclosure relates to an aqueous electroplating bath. The aqueous trivalent chromium bath may comprise:

trivalent chromium cations in an amount of 0.12-0.3 mol/l,

iron cations and/or nickel cations in an amount of 0.18-6.16 mmol/l, and

carboxylate ions in an amount of 1.2-7.4 mol/l, and

wherein the molar ratio of trivalent chromium cations to the carboxylate ions is 0.015-0.099, wherein the pH of the aqueous trivalent chromium bath is 2-6; and wherein the conductivity of the aqueous electroplating bath is 160-400 mS/cm.

The inventor surprisingly found out that it is possible to produce a hard chromium-based coating having a Vickers microhardness value of 900-2000 HV without the use of a heat treatment of the chromium-containing layer deposited from the electroplating bath by using the aqueous electroplating bath as disclosed in the current specification. The expression "heat treatment" should be understood in this specification, unless otherwise stated, as referring to subjecting the deposited chromium-containing layer to a heat treatment at a temperature of 300-1200° C. for a period of time that would result in the formation of chromium carbides in the chromium-based coating. Such a heat treatment may further change the crystalline structure of chromium. I.e. the method for producing the chromium-based coating may comprise the provision that the deposited chromium-containing layer is not subjected to a heat treatment to form a chromium-based coating having a Vickers microhardness value of 900-2000 HV. This provision may not, however, exclude e.g. dehydrogenation annealing.

In one embodiment, the chromium-based coating has a Vickers microhardness value of 1000-1900 HV, or 1100-1800 HV, or 1200-1700 HV, or 1300-1600 HV, or 1400-1500 HV. The Vickers microhardness may be determined according to standard ISO 14577-1:2015.

In one embodiment, the chromium-based coating may have a Taber index of below 1.5 mg/1000 RPM, or below 1.3 mg/1000 RPM, or below 1.2 mg/1000 RPM, or below 1.1 mg/1000 RPM as determined according to ASTM G195-18 (wheel CS10, 1000 g). Taber index indicates the wear resistance of the chromium-based coating. The smaller the value of the Taber index is, the better the wear resistance of the chromium-based coating.

In one embodiment, the crystal size of the chromium may be 7-40 nm, or 9-20 nm, or 11-16 nm. The crystal size of the chromium may be determined in the following manner:

Samples are measured with X-ray diffraction (XRD) in a 5 Grazing incidence (GID) geometry. In GID-geometry the X-rays are targeted on the sample with a small incident angle and held constant during the measurement. In this way, the X-rays can be focused on the surface layers of the sample, with the purpose of minimizing the signal from the substrate. 10 The measurements are performed on a 20 angular range of 30°-120°, with increments of 0.075°. A total measurement time for each sample is 1 h. The incident angle of X-rays is 4°. In addition to the samples, a corundum sample was measured with identical setup to measure the instrumental 15 broadening of diffraction peaks. The measurements are performed on a Bruker D8 DISCOVER diffractometer equipped with a Cu K $\alpha$  X-ray source. The X-rays are parallelized with a Gabel mirror, and are limited on the primary side with a 1 mm slit. An equatorial soller slit of 0.2° is used on the secondary side. The phases from the samples are identified from the measured diffractograms with DIFFRAC.EVA 3.1 software utilizing PDF-2 2015 database. The crystallite sizes and lattice parameters are determined from the samples by full profile fitting performed on TOPAS 4.2 software. The instrumental broadening is determined from the measurement of the corundum sample. The crystallite sizes are calculated using the Scherrer equation [see Patterson, A. (1939). "The Scherrer Formula for X-Ray Particle Size Determination". Phys. Rev. 56 20 (10): 978-982.], where the peak widths are determined with the integral breadth method [see Scardi, P., Leoni, M., Delhez, R. (2004). "Line broadening analysis using integral breadth methods: A critical review". J. Appl. Crystallogr. 37: 381-390]. The obtained values for lattice parameters are 25 compared to literature values from PDF-2 2015 database. The difference in measured values and literature values suggest the presence of residual stress within the coating.

In one embodiment, the chromium-based coating comprises 87-98 weight-%, or 92-97 weight-% of chromium. In 30 one embodiment, the chromium-based coating comprises 0.3-5 weight-%, or 1.0-3.0 weight-% of carbon. In one embodiment, the chromium-based coating comprises 0.1-11 weight-% of nickel and/or iron, or 1.1-8.2 weight-% of nickel and/or iron, or 1.5-6.2 weight-% of nickel and/or iron. I.e. the total amount of nickel and/or iron in the chromium-based coating may be 0.1-11 weight-%, or 1.1-8.2 weight %, or 1.5-6.2 weight %. In one embodiment, the chromium-based coating comprises 0-6 weight-%, or 0.1-5 weight-%, or 0.5-3.0 weight-% of nickel. In one embodiment, the 35 chromium-based coating comprises 0.1-5 weight-%, or 1.0-3.2 weight-%, of iron.

The amounts of different elements, such a chromium, iron, and nickel, in the chromium-based coating may be measured and determined with an XRF analyzer. The 40 amount of carbon in the chromium-based coating may be measured and determined with an infrared (IR) detector. An example of such a detector is the Leco C230 carbon detector.

The chromium-based coating may comprise also other 45 elements. The chromium-based coating may in addition comprise oxygen and/or nitrogen.

Usually, in order to achieve hard chromium-based coatings with a Vickers microhardness value of at least 900 HV, may have required the use of at least one heat treatment of the deposited chromium-containing layer at a temperature of 50 300-1200° C., when using an aqueous electroplating bath in which chromium is present substantially only in the trivalent form. The inventor surprisingly found out that such a heat

treatment may be omitted from the method when using the aqueous electroplating bath as defined in the current specification. By omitting this kind of heat treatment, one may be able to form a chromium-based coating that essentially lacks chromium carbides. The term "chromium carbide" is herein to be understood to include all the chemical compositions of chromium carbide. Examples of chromium carbides that may be present in the first layer are  $\text{Cr}_3\text{C}_2$ ,  $\text{Cr}_7\text{C}_3$ ,  $\text{Cr}_{23}\text{C}_6$ , or any combination of these. Such chromium carbides are usually formed into the chromium-based coating when the chromium-containing layer deposited on a substrate by electroplating from a trivalent chromium bath is subjected to at least one heat treatment at the temperature of 300-1200° C.

In this specification, unless otherwise stated, the terms "electroplating", "electrolytic plating" and "electrodeposition" are to be understood as synonyms. By depositing a chromium-containing layer on the substrate is herein meant depositing a layer directly on the substrate to be coated. In the present disclosure, the chromium-containing layer may be deposited through electroplating from an aqueous electroplating bath comprising trivalent chromium cations. In this connection, the wording electroplating "from an aqueous electroplating bath comprising trivalent chromium cations" is used to define a process step in which the deposition is taking place from an electrolytic bath in which chromium is present substantially only in the trivalent form.

As presented in the current specification, the aqueous electroplating bath may comprise:

trivalent chromium cations in an amount of 0.12-0.3 mol/l,  
iron cations and/or nickel cations in an amount of 0.18-6.16 mmol/l,  
carboxylate ions in an amount of 1.22-7.4 mol/l.

The molar ratio of trivalent chromium cations to the carboxylate ions is 0.015-0.099 in the aqueous electroplating bath. In one embodiment, the molar ratio of trivalent chromium cations to the carboxylate ions is 0.015-0.09, 0.03-0.08, or 0.065-0.075. The inventor surprisingly found out that the specified molar ratio of the trivalent chromium cations to the carboxylate ions has the added utility of enabling to omit the usually required heat treatment of the deposited chromium-containing layer to achieve a hard chromium-based coating.

Any soluble trivalent chromium salt(s) may be used as the source of the trivalent chromium cations. Examples of such trivalent chromium salts are potassium chromium sulfate, chromium(III)acetate, and chromium(III) chloride.

In one embodiment, the source of carboxylate ions is a carboxylic acid. In one embodiment, the source of the carboxylate ions is formic acid, acetic acid, or citric acid. In one embodiment, the source of the carboxylate ions is formic acid. In one embodiment, the source of the carboxylate ions is formic acid together with acetic acid and/or citric acid.

In one embodiment, the aqueous electroplating bath comprises trivalent chromium cations in an amount of 0.13-0.24 mol/l, or 0.17-0.21 mol/l.

The aqueous electroplating bath contains iron cations and/or nickel cations. The inventors surprisingly found that said cations may be needed in order to deposit the chromium-containing layer. The nickel ions may have the added utility of decreasing the potential needed in voltammetry. In one embodiment, the aqueous electroplating bath comprises iron cations in an amount of 0.18-3.6 mmol/l, or 0.23-0.4 mmol/l. In one embodiment, the aqueous electroplating bath comprises nickel cations in an amount of 0.0-2.56 mmol/l,

or 0.53-1.2 mmol/l. In one embodiment, the aqueous electroplating bath comprises iron cations and nickel cations in an amount of 0.18-6.16 mmol/l, or 0.76-1.6 mmol/l. In one embodiment, the aqueous electroplating bath comprises iron cations but not nickel cations. In one embodiment, the aqueous electroplating bath comprises nickel cations but not iron cations. In one embodiment, the aqueous electroplating bath comprises both iron cations and nickel cations.

In one embodiment, the aqueous electroplating bath comprises carboxylate ions in an amount of 2.0-6.0 mol/l, or 2.3-3.2 mol/l.

In one embodiment, the aqueous electroplating bath comprises a bromide ions in an amount of 0.15-0.3 mol/l, 0.21-0.25 mol/l. In one embodiment, the source of the bromide ions is selected from a group consisting of potassium bromide, sodium bromide, ammonium bromide, and any combination or mixture thereof. In one embodiment, the source of the bromide ions is potassium bromide, sodium bromide, or ammonium bromide. The use of the bromide, such as potassium bromide, may have the added utility of efficiently preventing the formation of hexavalent chromium at the anode of the electroplating system.

In one embodiment, the aqueous electroplating bath comprises ammonium ions in an amount of 2-10 mol/l, or 2.5-6 mol/l, or 3-3.4 mol/l. In one embodiment, the aqueous electroplating bath comprises ammonium ions in an amount of 0.18-1.5 mol/l, or 0.45-1.12 mol/l. The use of ammonium ions have the added utility of providing conductance to the aqueous electroplating bath. The use of ammonium ions have the added utility of forming a complex with the chromium. In one embodiment, the source of the ammonium ions is selected from a group consisting of ammonium chloride, ammonium sulfate, ammonium formate, ammonium acetate, and any combination or mixture thereof.

In one embodiment, the pH of the aqueous electroplating bath may be 2-6, or 3-5.5, or 4.5-5, or 4.1-5. The pH may be adjusted by including a base in the aqueous electroplating bath when needed. Ammonium hydroxide, sodium hydroxide, and potassium hydroxide may be mentioned as examples of bases that may be used for adjusting the pH of the aqueous electroplating bath. In one embodiment, the aqueous electroplating bath comprises ammonium hydroxide, sodium hydroxide, and/or potassium hydroxide. In one embodiment, the aqueous electroplating bath comprises a base in an amount of 0.5-3.1 mol/l, or 1.4-1.8 mol/l.

In one embodiment, the conductivity of the aqueous electroplating bath is 160-400 mS/cm, 200-350 mS/cm, or 250-300 mS/cm. The conductivity of the aqueous electroplating bath may be adjusted with the use of e.g. different salts for conductivity. Ammonium chloride, potassium chloride, and sodium chloride can be mentioned as examples of salts that may be used to adjust the conductivity. The conductivity may be determined e.g. in compliance with standard EN 27888 (water quality; determination of electrical conductivity (ISO 7888:1985)).

As is clear to the skilled person, the chromium-based coating may in addition to the materials presented above contain minor amounts of residual elements and/or compounds originating from manufacturing process, such as the electroplating process. Examples of such further elements are copper (Cu), zinc (Zn), and any compounds including the same.

The method and the chromium-based coating as disclosed in the current specification are well suited for protecting metal substrates from corrosion. In one embodiment, the corrosion resistance of the object is at least 24 h, or at least 48 h, or at least 96 h, or at least 168 h, or at least 240 h, or

at least 480 h. The corrosion resistance can be determined in accordance with standard EN ISO 9227 NSS (neutral salt spray) rating 9 or 10 (2017).

The thickness of the chromium-based coating can vary depending on the application where the object is to be used. The thickness of the chromium-based coating may depend on the number and thickness of the layers it comprises. In one embodiment, the thickness of the chromium-based coating is 0.05-200  $\mu\text{m}$ , or 0.5-100  $\mu\text{m}$ , or 0.3-5  $\mu\text{m}$ .

By a "substrate" is herein meant any component or body on which the chromium-based coating according to the present disclosure is coated on. Generally, the chromium-based coating according to the present disclosure can be used on variable substrates. In one embodiment, the substrate comprises or consists of metal, a combination of metals, or a metal alloy. In one embodiment, the substrate is made of steel, copper, nickel, iron, or any combination thereof. The substrate can be made of ceramic material. The substrate does not need to be homogenous material. In other words, the substrate may be heterogeneous material. The substrate can be layered. For example, the substrate can be a steel object coated by a layer of nickel, or nickel phosphorus alloy (Ni—P). In one embodiment, the substrate is a cutting tool, for example a cutting blade. In one embodiment, the substrate is a cutting tool comprising metal.

In one embodiment, the object comprising a chromium-based coating on a substrate does not comprise a layer of nickel. In one embodiment, the chromium-based coating does not comprise a layer of nickel. In one embodiment, the substrate does not comprise a layer of nickel.

In one embodiment, the object is a gas turbine, shock absorber, hydraulic cylinder, linked pin, joint pin, a bush ring, a round rod, a valve, a ball valve, or an engine valve.

In one embodiment, depositing the chromium-containing layer by subjecting the substrate to at least one electroplating cycle comprises subjecting the substrate to one, two, three, four, five, six, seven, eight, nine, or ten electroplating cycles. Each of the at least one electroplating cycles may be continued for 1 minute-4 hours, or 10-60 minutes, or 20-40 minutes, or for about 30 minutes. Each of the at least one electroplating cycles may be carried out at a current density of 50-300 A/dm<sup>2</sup>, or 80-250 A/dm<sup>2</sup>, or 110-200 A/dm<sup>2</sup>, or 120-180 A/dm<sup>2</sup>, or 130-170 A/dm<sup>2</sup>, or 140-150 A/dm<sup>2</sup>. The temperature of the aqueous electroplating bath may be kept at 25-70°C, or 40-50°C during the electroplating cycle(s). In one embodiment, the each of the at least one electroplating cycles is carried out at a deposition rate of 1.8-5  $\mu\text{m}/\text{minute}$ , or 2.0-4  $\mu\text{m}/\text{minute}$ , or 2.5-3.5  $\mu\text{m}/\text{minute}$ .

Each of the at least one electroplating cycles may be separated from another electroplating cycle in time so as to form at least two sublayers arranged one upon the other. In one embodiment, each of the electroplating cycles is separated from one another in time by stopping the electroplating process for a predetermined period of time. Each of the at least two electroplating cycles is separated from another electroplating cycle by at least 1 second, or at least 10 seconds, or at least 30 seconds, or at least 1 minute, or at least 5 minutes, or at least 10 minutes. In one embodiment, each of the at least two electroplating cycles is separated from another electroplating cycle by 0.1 milliseconds-3 minutes, or 1 second-60 seconds, or 10-30 seconds. In one embodiment, each of the at least two electroplating cycles is separated from another electroplating cycle by 0.5-10 minutes, or 2-8 minutes, or 3-7 minutes.

Different electroplating cycles may be separated from each other by stopping the current to pass through the aqueous electroplating bath. The substrate to be subjected to

the electroplating may be removed from the aqueous electroplating bath for a certain period of time and then put back into the bath for continued electroplating. The substrate to be subjected to electroplating may be removed from one trivalent chromium bath for a certain period of time and placed in another trivalent chromium bath for the sequential electroplating cycle to take place.

The method may further comprise polishing the surface of the chromium-based coating. Polishing or grinding the surface of the chromium-based coating, enables the formation of a smooth top surface. The method may comprise polishing the surface of the chromium-based coating to an Ra-value of below 0.6, or below 0.2. The roughness value (Ra-value) can be determined in accordance with EN ISO 4288:1998. The surface of the chromium-based coating may be polished to a roughness value required by the final application of the object.

The object disclosed in the current specification has the added utility of being well suited for applications wherein hardness of the object is relevant. The materials of the chromium-based coating have the added utility of providing the substrate a hardness suitable for specific applications requiring high durability of the object. The chromium-based coating has the added utility of protecting the underlying substrate from effects caused by the interaction with the environment during use. The chromium-based coating has the added utility of providing a good corrosion resistance. The chromium-based coating further has the added utility of being formed from trivalent chromium, whereby the environmental impact is less than when using hexavalent chromium. Further, the method as disclosed in the current specification has the added utility of being a safer production method for a chromium-based coating than if hexavalent chromium is used. Further, being able to omit the heat treatment of the chromium-containing layer while still providing a chromium-based coating with a high Vickers micro-hardness value, has the added utility of simplifying the production method and thus beneficially affects the production costs.

## EXAMPLES

Reference will now be made in detail to various embodiments, examples of which are illustrated in the accompanying drawings.

The description below discloses some embodiments in such a detail that a person skilled in the art is able to utilize the embodiments based on the disclosure. Not all steps or features of the embodiments are discussed in detail, as many of the steps or features will be obvious for the person skilled in the art based on this specification.

### Example 1—Preparing a Chromium-Based Coating on a Substrate

In this example different objects, each comprising a chromium-based coating on a substrate, were prepared.

Firstly, the substrates were pre-treated by cleaning the metal substrates, i.e. CK45 steel substrates, and providing thereon by electroplating and as a part of the substrate a nickel layer having a thickness of about 3-4  $\mu\text{m}$ . Thereafter the substrates were rinsed with water after which the chromium-based coating was formed on the substrate.

The aqueous electroplating bath comprised the following:

| Component                                                                               | Bath 1   | Bath 2                     | Bath 3                | Comparative |         |
|-----------------------------------------------------------------------------------------|----------|----------------------------|-----------------------|-------------|---------|
|                                                                                         | hardness | fast, high deposition rate | broad current density | Bath 4      | Bath 5  |
| Cr <sup>3+</sup> [mol/l]                                                                | 0.19     | 0.13                       | 0.19                  | 0.22        | 0.19    |
| Molar ratio of Cr <sup>3+</sup> to formate ion or equivalent amount of carboxylate ions | 0.068    | 0.080                      | 0.078                 | 0.097       | 0.051   |
| COOH <sup>-</sup> ions [mol/l]                                                          | 2.83     | 1.69                       | 2.46                  | 2.27        | 3.78    |
| KBr [mol/l]                                                                             | 0.23     | 0.23                       | 0.23                  | 0           | 0.23    |
| Fe [mmol/l]                                                                             | 0.27     | 0.11                       | 0.27                  | 0.18        | 0.27    |
| Ni [mmol/l]                                                                             | 0.0      | 2.98                       | 0.53                  | 0           | 0.53    |
| water                                                                                   | balance  | balance                    | balance               | balance     | balance |
| pH                                                                                      | 5        | 4.1                        | 5                     | 4.9         | 5.0     |
| Conductivity [mS/cm]                                                                    | 330      | 310                        | 270                   | 240         | 330     |
| Temperature of the bath during electroplating °C.                                       | 40       | 65                         | 45                    | 25          | 46      |
|                                                                                         |          |                            |                       |             | 45-60   |

The aqueous electroplating bath was subjected to a normal initial plating, after which it was ready for use.

A chromium-containing coating was deposited on each of the substrates by subjecting the substrates to electroplating cycles. The electroplating cycle was carried out for 10 minutes. Then the substrates with the chromium-containing layer were rinsed and polished to an Ra value of about 0.2.

The following properties and parameters of the chromium-based coating of the prepared objects were determined. The results are presented in the below table.

25 It is obvious to a person skilled in the art that with the advancement of technology, the basic idea may be implemented in various ways. The embodiments are thus not limited to the examples described above; instead, they may vary within the scope of the claims.

30 The embodiments described hereinbefore may be used in any combination with each other. Several of the embodiments may be combined together to form a further embodiment. An object, a method, or an aqueous electroplating bath disclosed herein, may comprise at least one of the embodi-

| Properties                                                    | Bath 1   | Bath 2         | Bath 3       | Bath 4 | Bath 5 | Comparative |
|---------------------------------------------------------------|----------|----------------|--------------|--------|--------|-------------|
|                                                               |          |                |              |        |        | bath        |
| Content/amount of Cr; Fe; and Ni (weight-%)*                  | 97; 3; 0 | 95.4; 0.6; 4.0 | 97; 1.2; 0.6 |        |        |             |
| Hardness (HV <sub>0.05</sub> )                                | 1750     | 1100           | 1700         | n/a    | n/a    | 700         |
| Deposition rate (μm/min)                                      | 3.15     | 6.01           | 3.9          | n/a    | 3.9    | 1.0         |
| Current density for the above properties (A/dm <sup>2</sup> ) | 150      | 200            | 150          | n/a    | 150    | 40          |

\*measured with an XRF analyzer that does not show the presence of carbon and scales the results to 100%

#### Example 2—Effect of the Current Density on the Hardness of the Chromium-Based Coating

In this example the effect of the current density during the electroplating was tested. The aqueous electroplating bath was a similar bath as bath 3 above in example 1. The results are presented in the below table.

| Current density (A/dm <sup>2</sup> ) | Crystal size (nm) | Hardness (HV) | Amount of Ni (weight-%)* | Amount of Fe (weight-%)* |
|--------------------------------------|-------------------|---------------|--------------------------|--------------------------|
| 50                                   | 4                 | 900           | 1.9                      | 2.7                      |
| 70                                   | 8                 | 890           | 1.6                      | 2.0                      |
| 120                                  | 12.4              | 1418          | 1.5                      | 1.6                      |
| 155                                  | 11.9              | 1394          | 1.2                      | 1.5                      |

\*measured with an XRF analyzer

50 ments described hereinbefore. It will be understood that the benefits and advantages described above may relate to one embodiment or may relate to several embodiments. The embodiments are not limited to those that solve any or all of the stated problems or those that have any or all of the stated benefits and advantages. It will further be understood that reference to 'an' item refers to one or more of those items. The term "comprising" is used in this specification to mean including the feature(s) or act(s) followed thereafter, without excluding the presence of one or more additional features or acts.

55 The invention claimed is:

60 1. An object comprising:  
a chromium-based coating on a substrate, wherein chromium of the chromium-based coating is electroplated from an aqueous electroplating bath comprising trivalent chromium cations, wherein the chromium-based

**11**

coating comprises 87-98 weight-% of chromium, 0.3-3 weight-% of carbon, and 0.1-11 weight-% of nickel and/or iron, and wherein the chromium-based coating has a Vickers microhardness value of 1000-2000 HV, and wherein the chromium-based coating does not 5 contain chromium carbide.

2. The object of claim 1, wherein the chromium-based coating has a Taber index of below 1.5 milligrams (mg)/1000 Rotations Per Minute (RPM), or below 1.3 mg/1000 RPM, or below 1.2 mg/1000 RPM, or below 1.1 mg/1000 10 RPM as determined according to ASTM G195-18, wherein the Taber index is calculated as  $((A-B)/1000)/C$ , wherein A is the initial weight, B is the final weight, and C is the amount of RPM.

3. The object of claim 1, wherein the crystal size of the 15 chromium is 7-40 nanometers (nm), or 9-20 nm, or 11-16 nm.

4. The object of claim 1, wherein the chromium-based coating has a Vickers microhardness value of 1000-1900 HV, or 1100-1800 HV, or 1200-1700 HV, or 1300-1600 HV, 20 or 1400-1500 HV.

5. The object of claim 1, wherein the object is a gas turbine, shock absorber, hydraulic cylinder, linked pin, joint pin, a bush ring, a round rod, a valve, a ball valve, or an engine valve. 25

**12**

\* \* \* \* \*